# EUROPEAN PATENT APPLICATION

(11) **EP 4 782 197 A1**
(43) Date of publication of application: **29.07.2026**
(21) Application number: 26151755.1
(22) Date of filing: 14.01.2026
(51) Int. Cl.: B32B 3/00, D06N 7/00

(54) **RECYCLABLE FLOOR COVERING ARTICLE COMPRISING CHEMICALLY MODIFIED POLYMER AND A METHOD OF PRODUCTION THEREOF**

(30) Priority: 14.01.2025 IN 202521003058
(71) Applicant: Welspun Living Limited, 400 013 Mumbai Maharashtra (IN)
(72) Inventor: Goenka, Dipali, 400013 Mumbai (IN); Dubey, Rahul, 400013 Mumbai (IN); Saluja, Deep Singh, 400013 Mumbai (IN)
(74) Representative: Nirwan, Prajwal

(57) **Abstract**

The present invention relates to recyclable floor covering article (100) and methods of making the same, wherein, the recyclable floor covering article comprises a single material, namely, a polymer (108), throughout its construction.The present disclosure specifically provides a recyclable floor covering article comprising (i) a primary backing (102) having a front face (102A) and a back face (102B), with a plurality of tufted pile yarn (104) tufted to the primary backing, extending from the front face of the primary backing and exposed at the back face of the primary backing, and (ii) a secondary backing (106) attached to the back face of the primary backing. The plurality of tufted pile yarn, the primary backing and the secondary backing are all made of the same polymer. The entire recyclable floor covering article is devoid of any adhesives or external recycling agents.

## Description

### TECHNICAL FIELD

The present invention relates to recyclable floor covering article and methods of making the same, wherein the recyclable floor covering article comprises a mono material throughout its construction. Specifically, the invention relates to a mono material floor covering article and a method of making the same by extrusion coating of a backing material comprising a mono material.

### BACKGROUND

Typically, a floor covering article, such as a carpet has composite structures comprising a primary backing layer and a secondary backing layer. The front face of the primary backing layer imparts the texture and appearance to the carpet, and is composed of tufted yarns. The primary backing secures these yarns in a layer of woven or non-woven, resilient thermoplastic material such as polyolefins, polyesters, nylon, latex, styrene butadiene/vulcanised rubber, and the like. The secondary backing layer of the carpet is primarily made of latex and/or styrene butadiene/vulcanised rubber to impart better performance, such as tuft strength, dimensional stability, ignition resistance, water resistance and the like, to the finished carpet. Sometimes the secondary backing is a single layer, but it is more common for the secondary backing to be made up of multiple layers. Commercially available carpets have an adhesive layer between the secondary backing layer and the primary backing layer for firmly affixing the tufted yarn. The adhesive layer is usually in the form of an adhesive coating. The adhesive coating is typically extruded over the primary backing layer, or application through liquified melt kiss rollers. Thereafter, the secondary backing layer is laminated over the adhesive coating to prepare the final product. In some cases, the carpets may consist of only primary backing and an adhesive layer with the adhesive layer acting as the secondary backing layer.

Nearly 90% of the carpets available in the market have secondary backing made from natural rubber and/or styrene-butadiene rubber, such as hydrogenated styrene-butadiene rubber or carboxylated styrene-butadiene rubber. According to *"*Carpet Laminating", Journal of Coated Fabrics. Volume 19, July 1989, pp. 35-52*,* the material most typically used for carpet back coating is styrene butadiene latex (SBR), usually a carboxylated SBR. These carpet backings comprise latex emulsion along with other inorganic fillers like calcium, in the form of limestone, and additives such as surfactants, penetrants, defoamers, dispersants, chelating agents, stabilizers, and thickeners etc. Latex incorporated secondary backing dominates the carpet industry due to their ability to impart better properties such as high tuft bind, and adhesion/delamination strength to the primary backing at a low cost. However, since latex is a thermosetting polymer, it is nearly impossible to recycle such latex based carpets. Further, latex based backing also deteriorates with age, or when it repeatedly comes in contact with water, thereby delaminating or peeling off from the primary backing.

Plasticizer migration is another major problem encountered with rubber based secondary backing. Most of the styrene-based carpet backings are rich in plasticizers that impart flexibility to the backing. These plasticizers may migrate from the secondary backing to the adhesive layer, as the adhesives usually have higher affinity for the plasticizer.

Recently, the carpet industry has also seen the emergence of polyurethane based secondary backing. However, their use is restricted due to the insulating effect of polyurethane which impacts the flammability performance of the overall finished carpet. However, polyurethane based backings are not economically feasible in comparison to latex backings.

Due to the drawbacks of latex and polyurethane, secondary backings made of thermoplastic polymers such as polyvinyl chloride (PVC), hot melt adhesives, polyolefins and bitumen have been developed. Many carpet manufacturers globally, for example, are now using bitumen and PVC in their carpet backing to predominantly cut costs. Further, backing made of PVC or polyolefin may additionally comprise a precoat of ethylene vinyl acetate (EVA). However, since these materials are not recyclable, this practice is harmful to the environment. Hotmelts have a higher tuft bind than latex, but they are costlier, become brittle in cold climates and do not provide impervious moisture barrier, while also having same issues as that of latex. The polyolefin-based backing is often thin, resulting in visible imperfections telescoping through the fibres.

The global textile waste crisis is exacerbated by non-recyclable rugs, carpets and area rugs. As discussed, the current rug constructions are predominantly made of composite materials (e.g., polypropylene face fibres, latex-based backings, and various adhesive layers) that are incompatible with existing recycling systems. As a result, these complex structures contribute significantly to landfill waste, with discarded carpets alone accounting for millions of tons of waste annually. With the world shifting towards sustainability, the focus is to develop products that are fully recyclable. There are several environmental disadvantages existing with the use of traditional latex, bitumen and thermoplastic polymers commercially used in carpet backings. Latex based backings are difficult to remelt at the end of the life cycle of the carpet, and even if melted, they may stick to the recycling apparatus or penetrate through the thermoplastic primary backing and the yarns, thereby contaminating them, making it impossible to separate the layers of carpet for further processing.

Materials such as PVC and bitumen are non-biodegradable and can last in the environment for up to 40 years. During its life cycle, PVC releases harmful chemicals like dioxins and phthalates into the air, water and land. Also, the EVA based precoats of polyolefins, hot melt adhesives and PVC release a lot of volatile organic compounds when heated during the recycling process. Further, EVA has a high environmental impact as more energy is needed to produce the polymer. *"*Hodgson, Alfred & Wooley, John & Daisey, Joan. (1993). Emissions of Volatile Organic Compounds from New Carpets Measured in a Large-Scale Environmental Chamber. Air & waste: journal of the Air & Waste Management Association. 43. 316-24. 10.1080/1073161X.1993.10467136*"* summarises the impact of VOC (volatile organic compunds) emissions from latex based, PVC and polyurethane based carpet backings.

Coupled with the above factors, the increasing cost and the plummeting availability of suitable landfills to discard the worn-out products, the carpet industry has experienced the need to find other alternatives. Several documents have addressed the issue of recyclability of carpet and/or carpet tiles.

WO1998038375**,** US9376769B2**,** WO9838374A2 disclose a carpet comprising (a) a primary backing which has a face and a back surface, (b) a plurality of fibers attached to the primary backing and extending from the face of the primary backing and exposed at the back surface of the primary backing, (c) an adhesive backing, (d) an optional secondary backing adjacent to the adhesive backing, and (e) at least one homogenously branched linear ethylene polymer. Methods of extrusion coating of at least one homogenously branched linear ethylene polymer onto the back surface of a primary backing to provide an adhesive backing are also disclosed. The entire carpet is made of 100% polyolefin to provide a recyclable carpet.

In another document WO2009086091**,** the carpet of WO1998038375 is modified to lower the growth tension of the carpet, i.e. to lower the thermal expansion of the adhesive in the direction of least resistance. This is achieved by providing an additional precoat of ethylene octene block copolymer, where the adhesive layer is extruded on the pre-coat. The adhesive layer of WO2009086091 thus comprises a tackifier, ethylene octene block copolymer and a filler, instead of the homogeneously branched linear ethylene polymer of WO1998038375. This only means more material and complexity at the time of recycling.

US2008280093 discloses a carpet like that disclosed in WO1998038375, but the adhesive material and the primary backing material are different, so they do not integrally fuse. The primary backing is made of polypropylene whereas the adhesive backing is made of polyethylene. However, carpets disclosed in US2008280093 are manufactured with different polymers in the backing fabric, yarn and the adhesive backing leading to difficulty in separation during the recycling process.

US11883984B2 discloses a recyclable single polymer floor covering article such as carpets or carpet tiles comprising (a) polyester pile yarn; (b) a spunbond nonwoven polyester primary backing layer; (c) a first layer of polyester hot melt adhesive having a viscosity of 3000 to 10,000 cps at 350°F, wherein the hot melt adhesive is comprised of at least 50 weight % recycled material; (d) a second layer of polyester hot melt adhesive having a viscosity that is three to five times higher than the viscosity of layer "c;" and (e) a polyester needle punch nonwoven secondary backing layer. The carpet is a single component (polyester) carpet product that can be easily recycled into fibres at the end life of the carpet.

Though the above-mentioned documents claim to produce a 100 percent recyclable carpet, they require an adhesive backing incorporated with additional polymeric materials other than the one used in primary backing, along with additional components such as tackifiers, fillers that are difficult to separate during recycling. While US11883984B2 discloses recyclable carpets that use polyester as the sole polymer throughout its construction, the major issue with such carpets is the use of hot melt adhesives for bonding the secondary backing to the primary backing. The incorporation of the hot melt adhesive requires special equipment, such as a hot melt gun to melt and apply, a process during which toxic fumes are released. Additionally, at the end of the life cycle of the carpet, the hot melt adhesive layers is required to be physically separated from the bonding materials before entering the recycle stream.

Waste resources utilization is of utmost importance today to promote sustainable development and minimize pollution. However, it remains a great challenge to reuse, recycle and turn post-consumer wastes into value-added products. It is therefore desirable to create products that are 100% recyclable, and with minimal intervention during the recycling process. Accordingly, there remains a need for a floor covering article that is developed from a single material which can be recycled without physical separation of the bonding materials, and which is environment friendly, user friendly, as well as does not create pollution during the manufacturing process.

While it may seem simple or obvious to eliminate the adhesives or external bonding materials, the use of a single material may not impart adequate dimensional stability and mechanical properties to the article, if these are avoided. Therefore, there is a need for alternate processes for improving the stability and mechanical properties of the article, without using external bonding agents or adhesives. As a result, one of the objectives of the present disclosure is to formulate processes that utilize reactive extrusion process as an alternative to use of adhesives.

WO1996029460A1 discloses tufted carpets having a face yarn, backing fabric, and adhesive binder each comprising a thermoplastic material selected from the group consisting of linear low-density polyethylene, low density polyethylene, ethylene copolymers, high density polyethylene, propylene random copolymers, polyamides, metallocene polyethylenes and syndiotactic polypropylene. The document discloses the application of a molten adhesive to the tufted primary via extrusion coating or laminating. Further, the document also discloses the use of functionalized polyolefin compatibilizers to aid in recycling at the end of its life, in case the tufted carpet is to be constructed from dissimilar thermoplastics, for example, nylon face yarns and polypropylene primary and secondary backings, as well as to reduce the overall viscosity of the thermoplastic adhesive and increase the wetting of the face yarns by the adhesive. These include maleated random-polypropylene copolymers sold as Fusabond MZ-278D by E. I. DuPont de Nemours & Company, maleated polyethylene wax sold by Eastman Chemicals, Inc. and ethylene-acrylic acid copolymers containing 3 to 20 percent acrylic acid, available from Exxon Chemicals. This document emphasizes the need for such compatibilizers for aiding in recyclability of tufted carpets constructed from dissimilar thermoplastics.

AU605596B2 discloses use of impact modifiers in reinforced polyester compositions containing an EPDM terpolymer grafted with 2% or more by weight of the said terpolymer with glycidyl methacrylate or glycidyl acrylate or a mixture thereof. ***S'anchez-Sol'is A et al,*** discloses the significance of grafting maleic anhydride in a PET- styrene butadiene polymer blend to increase the impact properties of the blend. *(*S'anchez-Sol'is A, Calderas F and Manero O. Influence of maleic anhydride grafting on the rheological properties of polyethylene terephthalate-styrene butadiene blends. Polymer 2001; 42(17): 7335*).* Similarly, Araujo et al, discloses that properties of polypropylene and PET blends can be improved by using elastomer functionalized by maleic anhydride (SEBS-g-MA) *(*Araujo, Luciana & Morales, Ana. (2018). Compatibilization of recycled polypropylene and recycled poly (ethylene terephthalate) blends with SEBS-g-MA. Polímeros. 28. 10.159010104-1428.03016*.).* These articles focus on blends of different polymers such as PP/PET, PET/SB polymers grafted with maleic anhydride, discussing improvements in impact properties, however these do not teach the effect of such modification on elasticity of the obtained polymer. None of the documents disclose use of the modified polymers in floor covering articles, carpets or rugs, and certainly do not suggest, motivate or teach single polymer carpets that are fully recyclable and sustainable.

The objective of the present invention is to not only improve recyclability of secondary backings of floor covering articles such as carpets, rugs, mats and the like by incorporating recyclable materials, but also to recycle the entire article at the end of its life cycle. The ability to recycle an article with a mono material is easier than multicomponent articles. At the same time, the secondary backings should be developed such that the functionality and mechanical properties of the components of the backings are preserved when used in extruding machines for manufacturing the backings. Further, as seen in the art, the incorporation of adhesive layer/backing makes the manufacturing and recyclability of these articles more complex.

Therefore, in light of the foregoing discussion, there exists a need to overcome the aforementioned drawbacks.

### SUMMARY

The aim of the present disclosure is to provide a recyclable floor covering article and a method of producing the same to provide a floor covering comprising a mono material in the primary and secondary backing layers. Therefore, addressing the issues of the prior art and the need for fully recyclable as well as functional floor covering articles with improved elasticity and flexibility, the present invention provides a floor covering comprising a mono material in the primary and secondary backing layers. The aim of the present disclosure is achieved by a recyclable floor covering article and a method of producing a recyclable floor covering article as defined in the appended independent claims to which reference is made to. Advantageous features are set out in the appended dependent claims.

The present disclosure provides a recyclable floor covering article comprising:
(i) a primary backing having a front face and a back face, with a plurality of tufted pile yarn extending from the front face of the primary backing, and
(ii) a secondary backing attached to the back face of the primary backing,
wherein the plurality of tufted pile yarn, the primary backing and the secondary backing are all made up of a polymer selected from the group comprising polyesters, polyolefins, nylon, and chemically modified forms thereof, such that the recyclable floor covering article is suitable for mechanical and/or chemical recycling at the end of its life, and wherein the recyclable floor covering article is free from adhesives and external processing agents.

The present disclosure also provides a method of producing recyclable floor covering article described above, the said method comprising:
(i) forming a non-woven primary backing layer using polymer fibers that are modified through spunbond process and tufting of yarn to provide the tufted primary backing layer;
(ii) separately treating the elastomer with a coupling agent through a reactive extrusion process to obtain a functionalized elastomer, and reacting the functionalized elastomer with the polymer in an extruder;
(iii) extrusion coating of the functionalised polymer (ii) on the back face of the primary backing (i), using a twin screw extruder.

The present disclosure provides a fully recyclable floor covering article that is made of mono material selected from the group comprising polyethylene terephthalate (PET), polylactic acid (PLA), polybutylene adipate terephthalate (PBAT) and polybutylene terephthalate (PBT), polycaprolactone (PCL), polyhydroxy butyrate (PHB) and polyhydroxy butyrate valerate (PHBV) and modifications of these polymers.

The floor covering articles of the present disclosure have a lower cost of production and have low impact on the environment as they are suitable for mechanical or chemical recycling.

It is an object of the present disclosure to provide a recyclable floor covering article comprising a single polymeric material throughout its construction.

Another object of the present disclosure is to provide a floor covering article which can be fully recycled at the end of its life, without segregation of its components.

Another object of the present disclosure is to provide a floor covering article free of latex.

Yet another object of the present disclosure is to provide a floor covering article free of adhesives and/or external recycling aids.

Still another object of the present disclosure is to provide a method for production of a recyclable floor covering article.

Yet another object of the present disclosure is to provide a process for manufacturing raw materials for use in preparing floor covering articles, through reactive extrusion.

Throughout the description and claims of this specification, the words "comprise", "include", "have", and "contain" and variations of these words, for example "comprising" and "comprises", mean "including but not limited to", and do not exclude other components, items, integers or steps not explicitly disclosed also to be present. Moreover, the singular encompasses the plural unless the context otherwise requires. In particular, where the indefinite article is used, the specification is to be understood as contemplating plurality as well as singularity, unless the context requires otherwise.

### BRIEF DESCRIPTION OF THE DRAWINGS

Embodiments of the present disclosure will now be described, by way of example only, with reference to the following diagrams wherein:
FIG. 1 is a schematic illustration of a recyclable floor covering article, in accordance with an embodiment of the present disclosure; and
FIG. 2 is an illustration of method of producing a recyclable floor covering article, in accordance with an embodiment of the present disclosure.

### DETAILED DESCRIPTION OF EMBODIMENTS

The following detailed description illustrates embodiments of the present disclosure and ways in which they can be implemented. Although some modes of carrying out the present disclosure have been disclosed, those skilled in the art would recognize that other embodiments for carrying out or practising the present disclosure are also possible.

Unless otherwise defined, all technical and scientific terms used herein have the same meaning as commonly understood by one of ordinary skill in the art to which this invention belongs.

The terminology used in the description of the invention herein is for the purpose of describing embodiments only and is not intended to be limiting of the invention.

Unless the context indicates otherwise, it is specifically intended that the various features of the invention described herein can be used in any combination.

Moreover, the present invention also contemplates that in some embodiments of the invention, any feature or combination of features set forth herein can be excluded or omitted.

All publications, patent applications, patents, and other references mentioned herein are incorporated by reference herein in their entirety for all purposes.

As used herein, "a," "an," or "the" can mean one or more than one.

In the following description, terms such as top, bottom, parallel and the like, are used solely for the purpose of clarity, and should not be taken as words of limitation.

The term 'floor covering article', as used herein, implies a textile article which comprises fibres made of yarn to cover surfaces which are used by people to walk on, or cover surfaces or use in areas like kitchen or bath rooms.. These articles include, but are not limited to, carpets, carpet tiles, rugs like area rugs, kitchen rugs and bath rugs, floor mats, bath mats and the like.

The term "single" and "mono" may be used interchangeably herein, to indicate the use of a single component or polymer in the making of the floor covering article, which is different from the recyclable floor covering article prepared with multi-components, i.e. with more than one type of polymers. For the purposes of the present disclosure, "mono-material" or "single material" or "single polymer" or "polymeric material" refers to a floor covering article in which all structural components are based on the same base polymer backbone, notwithstanding chemical modification, grafting or functionalisation that does not prevent joint recycling without separation.

The term "chemically modified forms thereof" refers to the chemically modified forms of the polymer that remain recyclable together without separation.

As discussed in the background of the present disclosure, conventional floor covering articles are produced using multi-material components such as polymer face fibres, latex backings, adhesives and the like, that nearly impossible to recycle due to numerous layers of different materials used in the construction, each of which needs to be processed differently. The primary objective of the present disclosure is to provide a 100% recyclable floor covering article comprising of a single material throughout its construction.

Accordingly, the present disclosure provides a recyclable floor covering article comprising : (i) a primary backing layer having a front face and a back face, with a plurality of tufted pile yarn tufted to the primary backing layer, extending from the front face of the primary backing and exposed at the back face of the primary backing layer, and (ii) a secondary backing layer attached to the back face of the primary backing layer. The recyclable floor covering article has a single material throughout its construction, i.e. the plurality of tufted pile yarn, the primary backing layer and the secondary backing layer comprises the same material such that the recyclable floor covering article is suitable for mechanical and/or chemical recycling at the end of its life. The recyclable floor covering article is completely free from adhesives and external recycling aids.

In one embodiment of the present disclosure, the single material used in the construction of the floor covering article is a polymer. The polymer is selected from the group comprising woven and non-woven polyesters, polyolefins and nylon. The polymer may be in virgin or recycled form, or a combination thereof.

In an embodiment, the polyesters may be selected from the group comprising polyethylene terephthalate (PET), polylactic acid (PLA), polybutylene adipate terephthalate (PBAT) and polybutylene terephthalate (PBT), polycaprolactone (PCL), polyhydroxy butyrate (PHB) and polyhydroxy butyrate valerate (PHBV) and combinations thereof.

In another embodiment, the polymer is a non-woven, recycled polypropylene. In yet another embodiment, the polymer is a non-woven, recycled nylon. In a preferred embodiment, the polymer is non-woven, recycled polyethylene terephthalate.

The primary backing layer of the floor covering article consists of a front face and a back face, with a plurality of tufted pile yarns extending from the front face of the primary backing and exposed at the back face of the primary backing layer. The term 'tufted pile yarn', as used herein, implies tufts of polymeric fibres or yarns that are inserted through a primary backing layer to create a pile of tufts that stand up from the base of the primary backing layer.

The primary backing layer serves as the foundational support for the floor covering article, providing strength and stability to the face fibres. The primary backing layer may be made of woven or non-woven polymers selected from the group comprising polyesters, polyolefins and nylon, which may be bio-based biodegradable, bio-based bio-nondegradable, petroleum-based degradable, petroleum-based non-degradable. The term "non-degradable" as used herein indicates degradation by chemical and/or mechanical intervention.

In a preferred embodiment, the primary backing layer is made of non-woven, recycled, polyethylene terephthalate.

The secondary backing layer of the floor covering article consists of the same polymer constituting the primary backing and yarn fibers. Secondary backings are ideally flexible, to provide support, stability and barrier between the recyclable floor covering article and the floor. Using polymer as a backing material for floor covering articles such as carpet is challenging due to its inherent properties and functional requirements. For instance, PET is naturally stiff and rigid, with low melt strength, making it less flexible as compared to traditional backing materials like latex. This rigidity complicates handling, installation, and achieving the soft, cushioned feel consumers often expect in carpets. Additionally, the hydrophobic nature and chemical inertness of the polymers hinder adhesion with face fibres or adhesives, risking delamination. Therefore, processing polymers for forming the secondary backing layer poses difficulties due to high melting point and thermal sensitivity, requiring precise temperature control to prevent material degradation during manufacturing. These polymers tend to shrink under heat or moisture adding to the complexity, as it can cause warping or instability in the final product. Achieving a single material recyclable carpet demands further innovation to ensure all additives and backings are compatible with recycling streams. Therefore, the flexibility and elastic properties of the floor covering article should not be impacted when adhesives are avoided. To obtain this objective, the polymer constituting the secondary backing is chemically modified using an elastomer. The elastomer monomers of block polymers, when added, react during the reactive extrusion process to impart elasticity to the polymer. Therefore, by chemically modifying the polymer, the polymer achieves the desired elastomeric properties, without introducing additives such as adhesives.

As used herein, the term 'chemically modified' implies modification of the polymer constituting the secondary backing layer of the floor covering article according to the present disclosure, to improve its mechanical and chemical properties. It must be noted that the chemical modification is carried out on the same polymer that is used in the primary backing layer, ensuring that while modified, the primary polymeric material used in the carpet is a single polymer. This helps ensure recycling of the carpet is efficient.

As used herein the term 'polymer composition' implies a composition comprising a polymer or the chemically modified polymer, an elastomer, compatibilizer and additives, used for preparation of the primary and secondary backing layers of the floor covering article.

In a preferred embodiment of the present disclosure, the secondary backing layer may be made of depolymerized recycled polyethylene terephthalate (PET) having high molecular weight in the range from about 6000g/mol to about 20000g/mol, and intrinsic viscosity in the range of about 0.8 dg/ml to about 0.11 dg/ml. The PET may be present in an amount ranging from about 80 wt% to about 99 wt% of the total polymer composition.

In another embodiment of the present disclosure, the secondary backing layer may be made of depolymerized recycled polypropylene having high molecular weight in the range from about 2,00,000 g/mol to about 6,00,000 g/mol, and melt flow index (MFI) in the range of about 3g/10 min to 25g/10 min. The polypropylene may be present in an amount ranging from about 80 wt% to about 99 wt% of the total polymer composition.

In yet another preferred embodiment of the present disclosure, the secondary backing layer may be made of depolymerized recycled nylon having high molecular weight in the range of about 10,000 g/mol to about 50,000g/mol, and relative viscosity (Rv) in the range of about 2g/ml to about 3g/ml. The nylon may be present in an amount ranging from about 80 wt% to about 99 wt% of the total polymer composition.

The elastomer used in the carpets according to the present disclosure is typically a styrene rubber, for example, a random or block copolymer containing styrene units and alkylene units, such as ethylene, propylene, isoprene or butylene. In an embodiment of the present disclosure, the elastomers may be selected from the group comprising styrene-ethylene-butylene-styrene, styrene-ethylene-butylene and styrene-ethylene ester based block copolymers. The elastomer may be present in an amount ranging from about 3% to about 8% by weight of the polymer composition

Blending of the elastomer and the polymer is achieved through use of coupling agents or compatibilizers to improve their compatibility. In one embodiment of the present disclosure, the compatibilizer is selected from the group comprising silane, carbodiimide, isocyanate, bisoxazolines, oxazolines, biscaprolactams, epoxides, anhydrides, phosphites and salts thereof. In a highly preferred embodiment of the present disclosure, the coupling agent is maleic anhydride.

In a preferred embodiment of the present disclosure, the elastomer is functionalised with the compatibilizer, wherein the functional groups present in the elastomer improve the compatibility of the elastomer with the polymer. In one embodiment, the functionalised elastomer may comprise the compatibilizer in an amount of about 1 wt% to about 10 wt % based on the total weight of the elastomer in the final polymer composition. In preferred embodiments, the compatibilizer may be present in an amount of about 2 wt% to about 8 wt% based on the total weight of the elastomer in the final polymer composition. In yet another embodiment, the compatibilizer may be present in an amount of about 3 wt% to about 5 wt% based on the total weight of the elastomer in the final polymer composition.

The polymer may be chemically modified with the functionalised elastomer through processes known in the art, including, but not limited to, chemical bonding, cross linking, hydrogen bonding and dipole-dipole interaction.

In a preferred embodiment of the present disclosure, secondary backing layer of the floor covering article is made of maleated styrene-ethylene-butylene-elastomer modified polypropylene.

In another preferred embodiment of the present disclosure, the secondary backing layer of the floor covering article is made of epoxidized nylon.

In a highly preferred embodiment of the present disclosure, the secondary backing layer is made of maleated styrene-ethylene ester-based block copolymer. In a most preferred embodiment of the present disclosure, the secondary backing layer is made of polyethylene terephthalate (PET) coupled with maleated- styrene-butadiene elastomer.

The secondary backing layer is preferably made by the process of reactive extrusion. Reactive extrusion is a method of chemically modifying polymers during the extrusion process. The process helps enhance the properties of the polymer, such that there is an improvement in tensile strength, impact resistance, and thermal stability of the polymer. The method employs the addition of a reactive monomer or compound to the polymer during extrusion. The monomer reacts with the polymer chains to form covalent bonds that change the properties of the polymer. Typical reactions that help modify the polymer during the reactive extrusion process include ionic polymerisation, reactive coupling and trans-esterification of the polymer. Real time chemical modification of the polymer is thus completed in the reactor.

In an embodiment of the present disclosure, the functionalised elastomer is present in an amount of not more than 25 wt% of the total polymer composition of the secondary backing. In preferred embodiments of the present disclosure, the functionalised elastomer is present in an amount of at least 10 wt%, preferably at least 15 wt%, more preferably at least 20 wt%, more preferably at least 25 wt%, based on the weight of the total polymer composition of the secondary backing layer.

The secondary backing layer composition may further contain one or more additives. Preferred additives may be one or more agents selected from the group comprising flow modifiers, plasticisers, antioxidants and antistatic agents or a combination thereof.

Flow modifiers may be selected from the group comprising polyols and benzyl benzoate in an amount ranging from about 1% to about 5% of the polymer composition.

Preferred plasticizers according to the present disclosure include plant oils and mineral oils. These oils improve the flexibility and softness of the polymer making them more pliable, especially for applications like rugs and carpets where a soft feel is desirable. Further, during processes like extrusion, these oils reduce the melt viscosity of the polymer, improving the flow characteristics of the polymeric composition and ensuring smooth processing and better mold filling, thereby resulting in a uniform and consistent final product. They also enhance the durability of the floor article by making it less prone to cracking or breaking under stress. The oils additionally act as a lubricant on the polymer surface during and after processing, leading to a smoother finish, reducing surface imperfections in the final product. Further, the oils can act as a heat stabilizer to some extent during high-temperature processes like extrusion. Any mineral oil or plant oil known in the art can be used according to the present disclosure. In one embodiment, the mineral oil used is paraffin oil. In another embodiment, the plant oil used is epoxidized soyabean oil. The oil may be used in an amount ranging from about 0.1% to about 5% by weight of the polymer composition.

Degradation of polymer upon exposure to oxygen is a naturally occurring phenomenon that is inevitable. To prevent such deterioration of the polymer constituting the backings, antioxidants may be added. The antioxidants ensure thermal stability of the polymer, thereby imparting dimensional stability over the broad range of temperature during manufacturing processes such as extrusion, and through the life cycle of the floor covering article. Typically, the most commonly used antioxidant in the manufacturing of the floor covering article of the present disclosure is triethylene glycol bis(3-tert-butyl-4-hydroxy-5-methylphenyl) propionate, in an amount ranging from about 0.01% to about 8.0% by weight of the polymer composition.

Antistatic agents are added to inhibit static generation when the floor covering article comes in contact with another surface. Antistatic agents may include polar and/or hydrophilic compounds conventionally used in the textile industry. These agents may be selected from the group including, but not limited to, polyethylene glycol esters, polyols, glycerol monostearate, long chain- alkyl phenols and the like. The anti-static agents may be used in an amount ranging from about 0.001% to about 1% by weight of the polymer composition.

The additives may be present in an amount ranging from about 0.01 wt% to about 10 wt% of the polymer composition constituting the secondary backing layer. In an embodiment, the additives may be present in an amount of at least 1 wt%, preferably at least 2 wt%, more preferably at least 5 wt % of the polymer composition.

In another embodiment of the present disclosure, there is provided a method of production of the floor covering article.

The method of producing the floor covering article of the present disclosure, comprises the following steps:
The pulverized polypropylene is combined with the styrene-ethylene-butylene elastomer and maleic anhydride-based compatibilizer in specified proportions. Benzyl benzoate is incorporated as a liquid phase additive to modify the viscosity and enhance melt flow behaviour. The mixture is fed into a reactive extruder where thermal and mechanical energy initiates a coupling reaction between SEB and maleic anhydride groups. The extrusion parameters (temperature, shear rate, and residence time) are optimized to achieve chemical bonding and homogeneity in a single step. The resulting material exhibits elastomeric properties suitable for carpet coatings, along with improved flow properties for seamless processing.

The front face of the primary backing layer may be constructed in any desired pattern or texture via tufting, which may be carried out on a conventional tufting machine known in the art. Conventional tufting equipment may be used at stitch spacing of from about 25 to 65 stitches per inch. The yarn used to produce the front face of the primary backing layer may have defined denier, based on the end-use of the floor covering article. The front face may have loop pile or cut pile construction or a combination thereof. For loop pile construction, the loops of yarn are formed during tufting, whereas for cut pile construction, the loops of yarn are either cut during or after tufting to develop single yarn ends.

The secondary backing layer can be developed as a laminate or extruded sheet on any machine conventionally known in the art.

Extrusion involves pushing a material through a die which is a small disk with an opening of specific size and shape. Extrusion results in formation of an object with a specific shape.

As discussed herein before, the objective of the disclosure is to eliminate the use of adhesives to achieve 100% recyclability of the floor covering article, without the requirement for physical separation of components prior to entering the recycling stream. To achieve this objective, the polymer composition constituting the secondary backing layer in formed as an extruded sheet in a conventional reactive extruder, such as a twin-screw extruder, which is commercially available. In a preferred embodiment of the present disclosure, the secondary backing layer may be applied as an extrusion coating onto the non-woven primary backing layer.

As used herein the term "extrusion coating" means a coating process in which a molten polymer composition as defined hereinbefore is extruded onto a primary backing. In extrusion coating technique, the polymer composition in powder form is heated in an extruder at a temperature above its melt temperature. The composition is then forced through the slot die to form a molten polymer sheet that is continuously drawn down onto the back face of the primary backing of the floor covering article. The polymeric composition of the secondary backing may be extruded onto the back face of the primary backing to form a thin film with thickness of about 300 GSM to about 1200 GSM, with thicknesses between about and 700 GSM to about 900 GSM being preferred. A person skilled in the art will understand that the thickness will depend on the desired end use of the floor covering article.

According to the preferred embodiment of the present disclosure, the secondary backing layer is extruded over the back surface of the primary backing layer via reactive extrusion. A major advantage of employing reactive extrusion in the production of the floor covering article is that it combines the chemical process of modification of the polymer constituting the secondary backing layer, as well as extruding over the primary backing, in a single step. The manufacturing process combines chemical processes and extrusion into a single step making the process relatively fast, cost effective and adhesive free, in comparison to the latex-based floor covering articles of the prior art.

In lamination process, secondary backing layer is applied onto the primary backing layer by developing the secondary backing layer as a solid sheet, followed by heating and elevating temperature of the sheet to laminate it over the back surface of the primary backing.

The primary and secondary backings are bonded to form a cohesive structure that meets industry standards for flexibility, durability, and functionality. The finished rug is made of a single polymer, ensuring it is fully recyclable in existing recycling streams and processes.

In an embodiment of the present disclosure, a recyclable PET floor covering article produced with the aforementioned method is provided. The recyclable floor covering article comprises: (i) a primary backing layer made of PET having a front face and a back face, with a plurality of tufted pile yarn made of PET, tufted to the primary backing layer, extending from the front face of the primary backing and exposed at the back face of the primary backing layer, and (ii) a secondary backing layer made of chemically modified PET attached as an extrusion coating to the back face of the primary backing layer. The chemically modified PET may consist of maleated styrene-ethylene ester based block copolymer, such that the PET is present in an amount ranging from about 80% to about 99% weight percentage of the total polymer composition, styrene-ethylene ester based block copolymer is present in an amount ranging from about 3% to about 8% by weight of the total polymer composition and maleic anhydride in an amount from about 3 wt% to about 5 wt% of the total polymer composition.

In another embodiment, a recyclable polypropylene floor covering article produced with the aforementioned method is provided. The recyclable floor covering article comprises: (i) a primary backing made of polypropylene having a front face and a back face, with a plurality of tufted pile yarn made of polypropylene tufted to the primary backing, extending from the front face of the primary backing and exposed at the back face of the primary backing, and (ii) a secondary backing made of chemically modified polypropylene attached as an extrusion coating to the back face of the primary backing. The chemically modified polypropylene may consist of maleated styrene-ethylene - butylene copolymer, such that the polypropylene is present in an amount ranging from about 80 wt% to about 99 wt% of the total polymer composition, styrene- ethylene - butylene copolymer is present in an amount ranging from about 3wt% to about 8 wt% of the total polymer composition and maleic anhydride in an amount from about 3wt % to about 5 wt% of the total polymer composition.

In another embodiment, a recyclable nylon floor covering article produced with the aforementioned method is provided. The recyclable floor covering article comprises: (i) a primary backing made of nylon having a front face and a back face, with a plurality of tufted pile yarn made of nylon tufted to the primary backing, extending from the front face of the primary backing and exposed at the back face of the primary backing, and (ii) a secondary backing made of chemically modified nylon attached as an extrusion coating to the back face of the primary backing. The chemically modified nylon is typically epoxidized nylon.

The floor covering article according to the present disclosure can be fully recycled at the end of its life, without segregation of its components. Conventionally known chemical and mechanical techniques such as depolymerization via methanolysis, glycolysis or hydrolysis; or melting, shredding and pelletizing can be employed for recycling the recyclable floor covering article. The recycled polymer resins can be reclaimed for preparing fresh floor covering article via melt spinning, extrusion coating, or other polymer processing technologies, thereby decreasing the reliance on virgin raw materials and enabling closed-loop recycling. According to the present disclosure, the recycling of the floor covering article may be carried out by melting, followed by solidification, shredding and further compounding for utilisation as melt spinning raw material for textile industry, or in the manufacturing of the reactive extruded compound for preparing the backing layer of a new floor covering article. Such efficiencies and advantages are not seen with conventional multi-component and latex floor covering articles, as the presence of the multi components and/or latex makes them ineligible for shredding and further processing. As a result, these cannot be fully recycled, and therefore add to the environmental burden.

Apart from recyclability, the use of single material also makes the recyclable floor covering article light weight compared to conventional articles developed from multi-material construction. Further, use of a single or mono material significantly reduces the production cost, and does not require adhesive backings that are commonly employed in the carpet backings of the prior art.

The mono material floor covering article of the present disclosure has several advantages over conventional article containing multi components and/or latex. A side-by-side comparison is depicted in the table below -

| **Parameter** | **Mono material articles of present disclosure** | **Latex or conventional floor covering articles** |
|---|---|---|
| **Material composition** | Single polymer (PET, PP, Nylon) | Multi component |
| **Recyclability** | Fully recyclable due to mono material construction | Difficult to recycle due to incompatible layers |
| **Durability** | High durability | Prone to delamination |
| **Weight** | Light weight due to mono material design | Heavier due to multi layer construction |
| **Manufacturing complexity** | Simpler process; no need for adhesive bonding | Complex process; requires separate manufacturing steps for face fiber and backing |
| **Odour and allergen concerns** | Minimal; no adhesives used | Latex can emit volatile organic compounds that can cause allergic reactions |
| **Cost efficiency** | Lower production cost | Higher due to multi component construction and processing |
| **Environmental impact** | Lower, due to recyclability and simpler disposal | Higher, due to non-recyclability and complex disposal |
| **End-of-life options** | Suitable for mechanical or chemical recycling | Limited recycling options, with inability to fully recycle; requires disposal in landfills or through incineration |

The mono-material, recyclable floor covering article according to the present disclosure retains the functional and aesthetic qualities demanded by consumers, while ensuring circularity in the product lifecycle.

The present disclosure is further illustrated by reference to the following examples which are for illustrative purposes only, and do not limit the scope of the invention in any manner.

### EXAMPLES

### EXAMPLE 1: Production of polyester recyclable carpet

### Example 1.1: Production of Primary backing

A primary backing layer was prepared using PET fibers that were modified through spunbond process to obtain a non-woven layer. Tufting of yarn was then carried out on this layer to provide the tufted primary backing layer.

### Example 1.2: Production of functionalised polymer-elastomer composition

PET granules obtained from reclaimed waste were converted into a powder having a particle size equivalent to 15 to 20 microns, using a pulverizer. Thereafter 2 Wt % of styrene butadiene elastomer was functionalised by reactive extrusion process using 1.5 wt% of maleic anhydride. The functionalisation was carried out as follows:
To the maleated styrene butadiene elastomer, 0.5 wt% of adhesive binder and 4 wt% of paraffin white oil was added at 230°C in a high speed melt, to obtain a mixture. A solution containing 3% of glycerol was then added to the mixture as a plasticizer. Herein, the term "adhesive binder" refers to a processing aid, a temporary rheology modifier, or a non-adhesive melt stabilizer.

This functionalised elastomeric mixture was then blended with the PET granules by feeding the granules through the side feeder of the extruder to obtain a final blend. To the blend, about 2% by wt of Triethylene glycol bis(3-tert-butyl-4-hydroxy-5-methylphenyl) propionate was added for thermal stability, and for ease in extrusion coating on the rugs and carpets. This ensures dimensional stability over the broad range of temperature used in the process.

### Example 1.3: Extrusion coating of Secondary backing onto the primary backing

The blend obtained in Example 1.2 was applied by extrusion coating on the back face of the primary backing obtained in Example 1.1, using a twin screw extruder.

The blend obtained in Example 1.2 was fed into a twin screw extruder for facilitating chemical reaction between the polymer and functionalised elastomer at molecular level and long strands were formed which in turn was converted to pellets having size of 0.125 to 0.3mm in the underwater pelletizer downstream equipment.

The obtained extruded secondary backing sheet was bonded to the primary backing to form the polyester carpet through extrusion coating process. The reaction parameters provided in Table 1 below were used. A precise temperature was controlled across 12 heating zones which resulted in a uniform, high-performance secondary backing as an extruded sheet.

**Table 1**

| **Extrusion Parameter** | **Quantity** |
|---|---|
| Output | 15kg/h |
| Screw speed | 15 rpm |
| Torque | 28%, 41Nm |
| Power | 1.2 Kw |
| Specific mechanical energy | 0.08KWh/kg |
| current | 20 amp |
| Melt pressure | 7 bar |
| Melt temperature | 245 C |
| Vacuum | 550mm/Hg |

### EXAMPLE 2: Production of polypropylene recyclable carpet

A recyclable polypropylene carpet was prepared using a process similar to that described in Example 1 above. The functionalised polymer-elastomer composition used for the polypropylene carpet was as follows -
Polypropylene (PP) : 60-80%
Styrene-Ethylene-Butylene (SEB) : 10-25%
Maleic Anhydride-Based Compatibilizer : 5-10%
Benzyl Benzoate : 1-5%

### EXAMPLE 3 : Recycling of the product

The carpet obtained in the examples above were subjected to recycling process. Yarn waste (PET or PP) was first subjected to discoloration and then put in a ball mill to facilitate hydrothermal reactions that facilitate cleavage of bonds. The individual monomer components were thus released, followed by addition to twin screw extruder along with other additives. Under water palletization of the blend was carried out to yield granules that were then subjected to melt spinning.

Recycling was carried out using chain extenders such as ECO-1120, which is a styrenic polymer with high content of GMA (glycidyl methacrylate), HPC-2108 or PET melt, all of which are helpful in breaking down the polymers in the recycling process.

The material was manually added in the hopper for preheating for 20 mins at 75°Celsius, while observing carefully to avoid degradation of the material. The yarn waste was then fed into a single screw extruder to create a melt, which was also accompanied by thermal and mechanical actions. Mineral oil was then added and extruded to create a uniform liquid melt. The liquid melt was then solidified with the application of water at room temperature to create a crystallization state. The crystallized material was shredded to create flakes which further were compounded by addition of chain extender concentrate and impact modifier. The end material thus obtained was useful for reuse in the preparation of the backing layer for the next batch of articles.

### DETAILED DESCRIPTION OF THE DRAWINGS

Referring to FIG. 1, illustrated is a schematic illustration of a recyclable floor covering article **100,** in accordance with an embodiment of the present disclosure. As shown, the recyclable floor covering article **100** comprises a primary backing **102** having a front face **102A** and a back face **102B,** with a plurality of tufted pile yarn **104** extending from the front face **102A** of the primary backing **102,** and a secondary backing **106** attached to the back face **102B** of the primary backing **102,** wherein the plurality of tufted pile yarn **104,** the primary backing **102** and the secondary backing **106** are all made up of a polymer **108** selected from the group comprising polyesters, polyolefins, nylon, and chemically modified forms thereof, such that the recyclable floor covering article **100** is suitable for mechanical and/or chemical recycling at the end of its life, and wherein the recyclable floor covering article **100** is free from adhesives and external processing agents.

Referring to FIG. 2, illustrated is flowchart depicting steps of a recyclable floor covering article, in accordance with an embodiment of the present disclosure. At step **202,** a non-woven primary backing layer is formed using polymer fibers that are modified through spunbond process and tufting of yarn to provide the tufted primary backing layer. At step **204,** the elastomer is separately treated with a coupling agent through a reactive extrusion process to obtain a functionalized elastomer, and the functionalized elastomer is reacted with the polymer in an extruder. At step **206,** the functionalised polymer (ii) is extrusion coated on the back face of the primary backing (i), using a twin screw extruder. It may be appreciated that "reacting the functionalized elastomer with the polymer" occurs in the same reactive extrusion process as of the separately treating of elastomer with the coupling agent through the reactive extrusion process.

Provided figures are merely examples, which should not unduly limit the scope of the claims herein. A person skilled in the art will recognize many variations, alternatives, and modifications of embodiments of the present disclosure.

## Claims

1. A recyclable floor covering article (100), comprising:
(i) a primary backing (102) having a front face (102A) and a back face (102B), with a plurality of tufted pile yarn (104) extending from the front face of the primary backing, and
(ii) a secondary backing (106) attached to the back face of the primary backing,
wherein the plurality of tufted pile yarn, the primary backing and the secondary backing are all made up of a polymer (108) selected from the group comprising polyesters, polyolefins, nylon, and chemically modified forms thereof, such that the recyclable floor covering article is suitable for mechanical and/or chemical recycling at the end of its life, and wherein the recyclable floor covering article is free from adhesives and external processing agents.

2. The recyclable floor covering article (100) as claimed in claim 1, wherein the polyester is selected from the group comprising polyethylene terephthalate (PET), polylactic acid (PLA), polybutylene adipate terephthalate (PBAT) and polybutylene terephthalate (PBT), polycaprolactone (PCL), polyhydroxy butyrate (PHB) and polyhydroxy butyrate valerate (PHBV) and modifications thereof.

3. The recyclable floor covering article (100) as claimed in claim 1, wherein the polyolefin is polypropylene.

4. The recyclable floor covering article (100) as claimed in claim 1 and claim 2, wherein the secondary backing (106) comprises a chemically modified polyethylene terephthalate (PET).

5. The recyclable floor covering article (100) as claimed in claim 1 and claim 3, wherein the secondary backing (106) comprises a chemically modified polypropylene.

6. The recyclable floor covering article (100) as claimed in claim 1, wherein the secondary backing (106) comprises a chemically modified nylon.

7. The recyclable floor covering article (100) as claimed in claims 4 to 6, wherein the polymer (108) is chemically modified by coupling with an elastomer.

8. The recyclable floor covering article (100) as claimed in claim 7, wherein the elastomer is selected from the group comprising styrene-ethylene-butylene-styrene, styrene-ethylene-butylene, and styrene-ethylene ester based block copolymers.

9. The recyclable floor covering article (100) as claimed in claim 7, wherein the coupling agent is selected from the group comprising silane, carbodiimide, isocyanate, bisoxazolines, oxazolines, biscaprolactams, epoxides, anhydrides and phosphites.

10. The recyclable floor covering article (100) as claimed in claim 9, wherein the coupling agent is maleic anhydride.

11. The recyclable floor covering article (100) as claimed in claim 1, wherein the secondary backing (106) further comprises additives selected from the group comprising flow modifiers, antioxidants, plasticizers, antistatic agents and combinations thereof.

12. The recyclable floor covering article (100) as claimed in claim 1, wherein the recyclable floor covering article is a carpet, rug, mat or a carpet tile.

13. A method of producing recyclable floor covering article as claimed in claim 1, the said method comprising:
(i) forming a non-woven primary backing layer using polymer fibers that are modified through spunbond process and tufting of yarn to provide the tufted primary backing layer;
(ii) separately treating the elastomer with a coupling agent through a reactive extrusion process to obtain a functionalized elastomer, and reacting the functionalized elastomer with the polymer in an extruder;
(iii) extrusion coating of the functionalised polymer (ii) on the back face of the primary backing (i), using a twin screw extruder.
